

Patented July 22, 1924.

1,502,425

# UNITED STATES PATENT OFFICE.

ROBERT HUGHES EVANS, OF DETROIT, MICHIGAN.

## HARDENING ALLOY FOR BEARING METALS AND PROCESS OF USING SAME.

No Drawing.

Application filed November 13, 1922. Serial No. 600,681.

To all whom it may concern:

Be it known that I, ROBERT H. EVANS, a citizen of the United States, residing at Detroit, in the county of Wayne and State 5 of Michigan, have invented certain new and useful Improvements in Hardening Alloys for Bearing Metals and Processes of Using Same; and I do hereby declare the following to be a full, clear, and exact description 10 of the invention, such as will enable others skilled in the art to which it appertains to make and use the same.

This invention relates to hardeners for bearing metals and to a process of making 15 suitably hardened bearing metals.

Its object is to facilitate the making of alloys for bearings especially in localities where crucibles and furnaces necessary for melting the more highly refractory ingredients 20 are not accessible and the ingredients are difficult to obtain.

Ordinary bearing metals of the babbitt type are composed of a relatively large proportion of lead,—which is readily procurable in all communities,—and a relatively small proportion of hardening ingredients such as antimony, tin, copper and bismuth,—which are not readily obtainable in smaller 25 communities. Antimony and copper have a relatively high melting point, and are not easily fused (particularly copper) with ordinary heating apparatus and melting containers. Furthermore, successful production 30 of a bearing metal alloy does not result from the mere mingling of the several ingredients in the correct proportions in the solid state and heating them together. For good results in making alloys for bearing metal it is essential to follow a certain procedure, 35 melting certain ingredients and adding others in definite order. It is not an easy matter for the ordinary mechanic or other person who wishes to line a bearing to produce the proper alloy, even if he has the necessary knowledge and ingredients, without suitable heating apparatus which may not be readily available at the locality where the work is to be done.

In order that a mechanic or other person 40 may easily and successfully produce a good bearing metal alloy of the proper composition in any locality with ordinary heating apparatus I have conceived of alloying the necessary hardening metals at the factory, thus rendering this hardening alloy readily

available as a distinct marketable product so that by purchasing this alloy any one can readily fuse it with the necessary quantity of lead in order to produce a successful bearing metal. This hardening alloy, although containing ingredients that cannot, separately, be melted at temperatures obtainable with ordinary heating means, is readily fusible in melted lead at a temperature obtainable with ordinary readily available heating means.

My invention therefore consists (1) in a hardening alloy as a distinct product composed of metals suitable for the purpose and (2) in the method of making bearing metals 70 which consists in fusing in and alloying with a quantity of melted lead the correct proportion of the previously formed hardening alloy.

The hardening alloy which is the subject 75 of this invention consists of (by weight) substantially seventy parts of antimony, twenty five parts of tin, three parts of copper and two parts of bismuth. In the preparation of this alloy it is necessary to first 80 fuse the copper with a small quantity of tin, in order to make an alloy having a lower melting point than copper, and to add the quantity of bismuth to reduce the melting point and prevent excessive shrinkage 85 of the ultimate bearing metal alloy. The copper fused with the small quantity of tin (say between one and two parts of the total hundred parts) and the bismuth are added to the melted antimony to produce 90 the hardening alloy.

In the process of making bearing metals substantially eighty parts of lead should be melted and substantially twenty parts of the described hardening alloy added to it. 95 The hardening alloy may be cut or divided into small pieces and introduced in a solid state into the molten lead and the particles of hardening alloy will readily fuse and alloy with the lead. The proportions 100 named are by weight.

In stating the proportion of the ingredients of the hardening alloy to be substantially seventy of antimony, twenty-five parts of tin, three parts of copper and two parts of bismuth in each one hundred parts by weight of the alloy, I mean to indicate that the maximum and minimum variations from these proportions should not be more than two parts of antimony, one part of tin, one 110

half part of copper and one half part of bismuth.

Thus, any mechanic or other person having this hardening alloy may make the highest grade bearing metal anywhere with facility because lead is readily procurable in any locality and melts at a relatively low temperature and the hardening alloy is readily fusible in molten lead or at the temperature at which lead melts.

Having described my invention what I claim and desire to secure by Letters Patent is:

1. As a distinct composition of matter a hardening alloy for bearing metals consisting of the following ingredients mixed

|          | Parts. | 20 |
|----------|--------|----|
| Antimony | 70     |    |
| Tin      | 25     |    |
| Copper   | 3      |    |
| Bismuth  | 2      |    |

2. The process of making bearing metals which consists in fusing a quantity of lead and adding to and alloying with the lead a previously prepared alloy consisting of antimony, tin, copper and bismuth, in substantially the proportions named.

In testimony whereof I affix my signature.

ROBERT HUGHES EVANS.